

Nov. 24, 1936.

W. D. HODSON

2,062,062

## CORDAGE LUBRICATION

Original Filed Dec. 6, 1935



Inventor,  
Walter D. Hodson  
By Dyanforth, Lee, Chatton & Wills,  
Attys.

## UNITED STATES PATENT OFFICE

2,062,062

## CORDAGE LUBRICATION

Walter D. Hodson, Beverly Hills, Ill.

Original application December 6, 1935, Serial No. 53,248. Divided and this application May 28, 1936, Serial No. 82,333

7 Claims. (Cl. 117—53)

This invention relates to lubricated cordage and more particularly to such cordage in which the yarn is formed about a porous fiber tube enclosing a viscous jelly-like lubricant.

5 In my Patent No. 2,028,155, issued January 21, 1936, and Patent No. 2,000,951, issued May 14, 1935, are disclosed lubricants for wire ropes and rope materials in general. The lubricants comprise a fibrous base of markedly higher lubricant 10 absorbing properties than the rope material, and a grease in proportions to produce a plastic jelly-like mass of lubricant. The fiber is normally asbestos.

A preferred grease may be prepared from a 15 viscous mineral oil, an aluminum soap, and an asphaltic or blown oil. For example, a suitable grease may be prepared of 39 parts of a heavy oil of 190—210 viscosity at 210° F., one part of aluminum oleate, and 50 parts of a blown oil having 20 approximately 100° melt point and a penetration in the order of 200 at 77° F. The fibrous base is incorporated in the lubricant in proportions depending upon the absorbing qualities of the base. A well ground, good quality asbestos may be used 25 in the proportions of 10 parts asbestos to 90 parts of grease, but normally, as set forth in my Patent No. 2,028,156, issued January 21, 1936, it is preferred to use mixtures of finely ground and coarsely ground asbestos in which generally about 30 25 parts of total asbestos is used for 75 parts of lubricant.

Such a lubricant may readily be incorporated in cordage material and thoroughly distributed therein by supplying the lubricant in the form of 35 a thin tube of material surrounded by a lubricant permeable fabric rapidly disintegrated by the lubricant, and forming the cordage yarn about such tube.

The invention is illustrated in the drawing, in 40 which—

Fig. 1 is a sectional elevation of a nipper assembly or spinning die for the formation of yarn; Figs. 2—8, inclusive, represent progressive changes in the shape of the tube forming die; and Fig. 9 45 is a cross section of a tube of lubricant.

Fig. 1 shows a conventional form of spinning die 10, in which a ribbon-forming passage or die 11 has been drilled. The ribbon-forming passage originally has a cross section, as shown in Fig. 4 50 and into this a flat fabric ribbon 12 is introduced. The shape of the passage 11 gradually changes in cross section to bend the edges of the ribbon 12 gradually about until they have substantially met. These changes are illustrated in Figs. 3 to 6. At 55 a point in the die just prior (in the direction of

movement of the ribbon 12) to the junction of the edges, a lubricant-feeding device 13 opens into the die adapted to feed lubricant between the edges of the fabric. This lubricant feeder is preferably flexibly mounted on the member 14 to 5 allow for movement thereof. After passing the lubricant-feeding device, the shape of the die changes to an ellipse, and then to a circle, to force the edges of the ribbon together and into overlapping position. To facilitate overlapping, the 10 die must be shaped to raise one edge of the fabric slightly over the other at a point just prior to overlapping.

At the exit 15 of the die 11 the ribbon is caught in the fibers 16 at a point just before they are 15 twisted into the yarn 17.

The fibrous material of such a ribbon is of a material, preferably paper, which is highly absorbent with respect to the lubricant employed and is rapidly disintegrated by absorbed lubricant. The result is that lubricant is not thrown off in the spool box of the spinning machine, but is immediately available for distribution into the fibers and is forced into even distribution by future twisting operations and by the disintegration 20 of the fabric. 25

A ribbon may be used which is not absorbent for or disintegrated by the lubricant, but which acts as an open mesh retainer therefor until the pressure of subsequent twisting operations in the 30 manufacture of strands and rope squeezes the lubricant through the pores of the fabric and into the cordage material. In such case, any method of feeding may be employed, and the tube may be loaded with grease in advance. 35

In practice, the width of the ribbon 12 is slightly more than enough to form a tube of the desired diameter. For example, with a tube having a diameter of one-sixteenth inch, the ribbon may be about one-fourth inch. The tube normally will 40 have a diameter less than one-eighth inch, but it will, of course, depend upon the size of the cordage and its absorptiveness.

The term "lubricant permeable fabric", as used 45 herein, applies both to porous fabrics and to fabrics which are rapidly disintegrated by the lubricant and become permeable after such disintegration.

The foregoing detailed description has been 50 given for clearness of understanding only, and no unnecessary limitations should be understood therefrom, but the appended claims should be construed as broadly as permissible, in view of the prior art.

This application is a division of my copending application Serial No. 53,248.

I claim:

1. As an article of commerce, a tube of small diameter and having porous fabric walls and being substantially filled with a viscous jelly-like lubricant.
2. Cordage yarn comprising rope fibers formed into yarn about a porous fiber tube enclosing a viscous jelly-like lubricant.
3. As an article of commerce, a tube of small diameter having walls of a lubricant-permeable fabric, said tube being substantially filled with a cordage lubricant.
4. An article as set forth in claim 3, in which

the lubricant comprises a grease and a highly absorbent fibrous material.

5. Cordage yarn comprising rope fibers formed into yarn about a porous fiber tube enclosing a plastic cordage lubricant.

6. Cordage yarn comprising rope fibers formed into yarn about a porous fibered tube enclosing a viscous lubricant comprising a grease and a fibrous material markedly more absorbent than the cordage.

10 7. Cordage yarn comprising rope fibers formed into yarn about a porous fibered tube enclosing a viscous jelly-like cordage lubricant and fibrous material markedly more absorbent than the cordage.

15 WALTER D. HODSON.